# EUROPEAN PATENT APPLICATION

(11) **EP 4 759 956 A1**
(43) Date of publication of application: **17.06.2026**
(21) Application number: 24851093.5
(22) Date of filing: 08.08.2024
(51) Int. Cl.: C22C 38/02, C22C 38/18, C22C 38/46, C22C 38/04, C21D 8/10

(54) **HIGH-STRENGTH AND CARBON DIOXIDE CORROSION-RESISTANT TUBING AND CASING AND MANUFACTURING METHOD THEREFOR**

(30) Priority: 09.08.2023 CN 202310997786
(71) Applicant: BAOSHAN IRON & STEEL CO., LTD., Shanghai 201900 (CN)
(72) Inventor: Yuan, Kaijie, Shanghai 201900 (CN); Dong, Xiaoming, Shanghai 201900 (CN); Gao, Zhan, Shanghai 201900 (CN); Lu, Xiaoqing, Shanghai 201900 (CN)
(74) Representative: Kuhnen & Wacker Patent- und Rechtsanwaltsbüro PartG mbB
(86) International application number: PCT/CN2024/110665
(87) International publication number: WO 2025/031448

(57) **Abstract**

Disclosed in the present invention is a high-strength and carbon dioxide corrosion-resistant tubing and casing, comprising Fe and inevitable impurities, and further comprising the following chemical elements: C: 0.10-0.20%, Si: 0.10-0.80%, Mn: 0.10-1.50%, Cr: 3-5%, Mo: 0.10-0.70%, Al: 0.01-0.10%, V: 0.10-0.20%, Ni: 0.1-1.0%, Ce: 0.002-0.01%, and La: 0.002-0.01%. Correspondingly, further disclosed in the present invention is a manufacturing method for the high-strength and carbon dioxide corrosion-resistant tubing and casing. In the present invention, by means of reasonable component design of chemical elements, the tubing and casing having both ultrahigh strength and excellent carbon dioxide corrosion resistance can be obtained.

## Description

### Technical Field

The present invention relates to a steel material and a manufacturing method therefor, and particularly to a petroleum casing pipe and a manufacturing method therefor.

### Background

In the development process of petroleum and natural gas, corrosion issues often lead to significant economic losses and even catastrophic consequences. Currently, severe CO₂ corrosion problems exist in many oilfields.

Although extensive research has been conducted both domestically and internationally, and CO₂ corrosion-resistant materials such as 13Cr steel and high-corrosion-resistance Ni-based alloys have been developed, these materials contain large amounts of precious metal elements such as Cr, Ni, and Mo, resulting in a substantial increase in the cost of steel tubes.

In the existing technology, most alloy steels used for resisting CO₂ corrosion (or combined corrosion of CO₂ + H₂S + Cl⁻ simultaneously) belong to medium-alloy or high-alloy composition systems such as 13Cr. The low-alloy 3Cr series corrosion-resistant petroleum casing pipes have relatively low strength, failing to meet the requirements of the 110 ksi steel grade and above.

For example, the Chinese patent document with Publication No. CN101899621A, published on December 1, 2010, and titled "3Cr Seamless Steel Tube and Its Manufacturing Method" has the following chemical composition: C: 0.1-0.2%, Si: 0.1-0.5%, Mn: 0.3-0.8%, Cr: 2-4%, Mo: 0.3-0.6%, Ti: 0.0024-0.024%, Al: 0.01-0.04%, P ≤ 0.03%, S ≤ 0.03%, with the balance being Fe and unavoidable impurities. By adopting a quenching and tempering heat treatment process, a yield strength of ≥ 552 MPa (i.e., 80 ksi) is achieved.

Another example is the Chinese patent document with Publication No. CN103602903A, published on February 26, 2014, and titled "High-Strength Oil Well Pipe Resistant to Carbon Dioxide Corrosion and Its Manufacturing Method". Its chemical composition is: C: 0.30-0.42%, Si: 0.10-1.0%, Mn: 0.80-1.5%, Cr: 0.5-1.5%, V: 0.21-0.4%, Al: 0.01-0.10%, N: 0.031-0.05%, P ≤ 0.015%, S ≤ 0.005%, with the balance being Fe and unavoidable impurities. The V/N ratio is controlled within the range of 6-11, and by adopting a normalizing process, the mechanical properties reach the 95 ksi steel grade and above.

### Summary

One of the objectives of the present invention is to provide a high-strength petroleum casing pipe resistant to carbon dioxide corrosion. Through a rational design of chemical element composition, the petroleum casing pipe can achieve both ultra-high strength and good carbon dioxide corrosion resistance.

To achieve the above objective, the present invention provides a high-strength petroleum casing pipe resistant to carbon dioxide corrosion, which comprises Fe and unavoidable impurities, and further comprises the following chemical elements in the following mass percentages:
C: 0.10-0.20%, Si: 0.10-0.80%, Mn: 0.10-1.50%, Cr: 3-5%, Mo: 0.10-0.70%, Al: 0.01-0.10%, V: 0.10-0.20%, Ni: 0.1-1.0%, Ce: 0.002~0.01%, and La: 0.002~0.01%.

Correspondingly, the present invention further provides a high-strength petroleum casing pipe resistant to carbon dioxide corrosion, wherein the mass percentage contents of each element of the high-strength petroleum casing pipe resistant to carbon dioxide corrosion are as follows:
C: 0.10-0.20%, Si: 0.10-0.80%, Mn: 0.10-1.50%, Cr: 3-5%, Mo: 0.10-0.70%, Al: 0.01-0.10%, V: 0.10-0.20%, Ni: 0.1-1.0%, Ce: 0.002~0.01%, La: 0.002~0.01%, and a balance of Fe and other unavoidable impurities.

In general, to improve the CO₂ corrosion resistance of a material, a certain amount of Cr is usually added to form a dense corrosion film for protecting the base material. However, Cr elements tend to combine with C elements to form carbides such as C₂₃C₆ and C₇C₃, making it impossible to form a Cr(OH)₃ corrosion film with anion selectivity. Therefore, the present invention adopts a low-carbon composition design to reduce the content of Cr carbides, thereby promoting the enrichment of Cr in the corrosion film, enhancing the stability of the corrosion film, and ultimately improving the corrosion resistance. Meanwhile, Ce and La elements are added. On one hand, these elements have strong affinity with elements such as O and S, enabling deep deoxidation and forming rare earth compounds that facilitate impurity removal during smelting. This reduces the content of coarse inclusions and prevents the formation of pitting pits at the locations of large inclusions. On the other hand, rare earth elements reduce the degree of undercooling during crystallization, leading to structure refinement in the solidification process. Through rare earth modification, uniformly dispersed and fine rare earth inclusion particles are formed, which can not only serve as nucleation cores for the second phase but also produce a grain boundary pinning effect. This is beneficial for grain refinement and the improvement of comprehensive properties. In addition, through the microalloying composition design of multiple elements including V, Ni, and Nb, the present invention can achieve a high yield strength of 140 ksi, and an improved corrosion resistance, and the collapse resistance of the casing pipe is also enhanced, thereby significantly extending the service life of the casing tube.

Specifically, in the high-strength petroleum casing pipe resistant to carbon dioxide corrosion according to the present invention, the design principles of each chemical element are as follows:
C: In the high-strength petroleum casing pipe resistant to carbon dioxide corrosion according to the present invention, C is a primary solid solution strengthening element that can improve the strength of the steel. However, an excessively high content of C will worsen segregation, reduce toughness, and the formation of carbides will impair corrosion resistance. Therefore, the C content in the present invention is controlled within the range of 0.10-0.20%.
Si: In the high-strength petroleum casing pipe resistant to carbon dioxide corrosion according to the present invention, Si acts as a deoxidizer. It exerts a strong solid solution strengthening effect on ferrite, improving hardenability, temper resistance, and yield strength. Nevertheless, an excessively high Si content will deteriorate the toughness and processability of the steel. Thus, the Si content in the present invention is controlled within the range of 0.10-0.80%.
Mn: In the high-strength petroleum casing pipe resistant to carbon dioxide corrosion according to the present invention, Mn is one of the important alloying elements. It significantly enhances the hardenability of the steel and promotes the formation of martensite to ensure strength. However, an excessively high Mn content tends to cause adverse effects such as grain coarsening and structural segregation. Therefore, the Mn content in the present invention is controlled within the range of 0.10-1.50%.
Cr: In the high-strength petroleum casing pipe resistant to carbon dioxide corrosion according to the present invention, Cr is the main alloying element for improving corrosion resistance and can also increase the hardenability of the steel. Hence, the Cr content in the present invention is controlled within the range of 3-5%.
Mo: In the high-strength petroleum casing pipe resistant to carbon dioxide corrosion according to the present invention, Mo has a strong ability to inhibit the transformation of austenite to pearlite, can suppress temper brittleness, and forms dispersed special carbides at relatively high tempering temperatures to improve strength. Based on this, the Mo content in the present invention is controlled within the range of 0.10-0.70%.
Al: In the high-strength petroleum casing pipe resistant to carbon dioxide corrosion according to the present invention, Al is mainly used for deoxidation and grain refinement, and it has a significant solid solution strengthening effect. On this basis, the Al content in the present invention is controlled within the range of 0.01-0.10%.
V: In the high-strength petroleum casing pipe resistant to carbon dioxide corrosion according to the present invention, V is a strong carbide and nitride-forming element. It improves the temper resistance of the steel, exerts a strong secondary hardening effect, and when dissolved in ferrite, provides an extremely strong solid solution strengthening effect. However, an excessively high V content tends to form coarse V(C,N), which impair toughness. Therefore, the V content in the present invention is controlled within the range of 0.10-0.20%.
Ni: Ni has a certain solid solution strengthening effect and can improve corrosion resistance. In the high-strength petroleum casing pipe resistant to carbon dioxide corrosion according to the present invention, the combined use of Ni with Cr and Mo can enhance the thermal strength and corrosion resistance of the steel. Based on this, the Ni content in the present invention is controlled within the range of 0.1-1.0%.
Ce and La: In the high-strength petroleum casing pipe resistant to carbon dioxide corrosion according to the present invention, trace additions of Ce and La are used for grain refinement and toughness improvement. However, an excessively high content of these elements tends to form coarse oxides or oxysulfides. Therefore, both the Ce content and La content in the present invention are controlled within the range of 0.002-0.01%.

Further, in the high-strength petroleum casing pipe resistant to carbon dioxide corrosion according to the present invention, the mass percentage contents of each chemical element may further satisfy at least one of the following items:
Si: 0.1-0.4%;
Mn: 0.2-1.0%;
Mo: 0.4-0.6%;
Al: 0.01-0.04%;
Ni: 0.1-0.5%;
Ce: 0.002-0.008%; and
La: 0.002-0.005%.

Further, the high-strength petroleum casing pipe resistant to carbon dioxide corrosion according to the present invention further comprises 0 < Nb ≤ 0.15wt%.

Nb has a strong solid solution strengthening effect and can refine grains. Trace addition of Nb can improve the strength of the steel without affecting its plasticity and toughness. Based on this, in some embodiments of the present invention, its content is controlled to 0 < Nb ≤ 0.15wt%, for example, 0.01wt% ≤ Nb ≤ 0.15wt%.

Further, among the unavoidable impurities in the high-strength petroleum casing pipe resistant to carbon dioxide corrosion according to the present invention: P ≤ 0.015%, S ≤ 0.008%, and N ≤ 0.008%.

Still further, P ≤ 0.012%, S ≤ 0.005%, and N ≤ 0.006% are controlled.

In the above technical solution of the present invention, P, S, and N are all harmful impurity elements. Among them, P and S segregate severely in steel, which is unfavorable to plasticity and toughness. N has no significant strengthening effect; it forms nitrides that impair the strengthening effect of microalloying elements, and it is prone to cause age hardening in low-carbon steel, reducing plasticity and toughness. Therefore, in order to obtain steel with better performance and higher quality, the contents of P, S, and N should be reduced as much as possible under technically feasible conditions.

Further, the matrix microstructure of the high-strength petroleum casing pipe resistant to carbon dioxide corrosion according to the present invention is tempered sorbite.

Further, the grain size of the high-strength petroleum casing pipe resistant to carbon dioxide corrosion according to the present invention is Grade 10 or above. In some embodiments, the grain size of the high-strength petroleum casing pipe resistant to carbon dioxide corrosion according to the present invention is Grade 10-11.

Further, in the high-strength petroleum casing pipe resistant to carbon dioxide corrosion according to the present invention, the percentage by quantity of large inclusions with an average diameter greater than 5µm in all inclusions is < 6%. In some embodiments, the percentage by quantity of large inclusions with an average diameter greater than 5 µm in all inclusions is ≥ 3% and < 6%.

Further, the Cr content in the corrosion product film of the high-strength petroleum casing pipe resistant to carbon dioxide corrosion according to the present invention is higher than 13wt%. In some embodiments, the Cr content in the corrosion product film is > 13 wt% and ≤ 21 wt%. The corrosion product film is formed under the corrosion environment conditions of a temperature of 60°C, a CO₂ partial pressure of 1 MPa, and a NaCl concentration of 20 g/L.

Further, the properties of the high-strength petroleum casing pipe resistant to carbon dioxide corrosion according to the present invention meet the following requirements: a yield strength of 965-1173 MPa, a tensile strength ≥ 1034 MPa, and a transverse Charpy impact energy at 0°C ≥ 80 J.

In some embodiments, the tensile strength of the high-strength petroleum casing pipe resistant to carbon dioxide corrosion according to the present invention is 1034~1300 MPa.

In some embodiments, the transverse Charpy impact energy at 0°C of the high-strength petroleum casing pipe resistant to carbon dioxide corrosion according to the present invention is 80~200 J.

In some embodiments, the elongation after fracture of the high-strength petroleum casing pipe resistant to carbon dioxide corrosion according to the present invention is 18-25%.

Further, the uniform corrosion rate of the high-strength petroleum casing pipe resistant to carbon dioxide corrosion according to the present invention is ≤ 2.5 mm/a (e.g., 0.5~2.5 mm/a) under the corrosion environment conditions of a temperature of 60°C, a CO₂ partial pressure of 1 MPa, and a NaCl concentration of 20 g/L.

Accordingly, another object of the present invention is to provide a manufacturing method for the aforementioned high-strength petroleum casing pipe resistant to carbon dioxide corrosion, which has a simple process and low production cost.

To achieve the above object, the present invention provides a manufacturing method for the aforementioned high-strength petroleum casing pipe resistant to carbon dioxide corrosion, comprising the following steps:
(1) smelting and continuous casting to obtain a pipe billet;
(2) heating, piercing, rolling, and sizing;
(3) quenching: heating to a quenching temperature of 880~920°C, holding for 30~60 minutes, followed by water quenching;
(4) tempering: heating to a tempering temperature of 550~650°C, with a holding time of 45~75 minutes.

Further, in step (1) of the manufacturing method according to the present invention, during the casting process, the superheat degree of molten steel is controlled to be ≤ 30°C (e.g., 15~30°C), and the continuous casting speed is controlled at 2.0 m/min or lower (e.g., 1.8-2.0 m/min).

Further, in step (2) of the manufacturing method according to the present invention, the pipe billet is heated to a soaking temperature of 1200~1250°C and held for 100-300 minutes.

Further, in step (2) of the manufacturing method according to the present invention, the piercing temperature is controlled at 1150~1250°C.

Further, in step (2) of the manufacturing method according to the present invention, the finishing rolling temperature is controlled at 900~1000°C.

Further, in step (2) of the manufacturing method according to the present invention, the sizing temperature is controlled at 850-950°C.

Further, in step (4) of the manufacturing method according to the present invention, air cooling is performed after holding.

The high-strength petroleum casing pipe resistant to carbon dioxide corrosion and its manufacturing method according to the present invention have the following advantages and beneficial effects:
The high-strength petroleum casing pipe resistant to carbon dioxide corrosion according to the present invention adopts a low-carbon composition design, with appropriate addition of Cr element, as well as a design of Ni, Mo, V, Ce, and La elements, enabling the produced petroleum casing pipe to have both high strength and good corrosion resistance.

In some embodiments, the yield strength of the high-strength petroleum casing pipe resistant to carbon dioxide corrosion according to the present invention is 965-1173 MPa (reaching 140 ksi), the tensile strength is ≥ 1034 MPa, and the transverse Charpy impact energy at 0°C is ≥ 80 J, exhibiting excellent mechanical properties.

In some embodiments, the uniform corrosion rate of the high-strength petroleum casing pipe resistant to carbon dioxide corrosion according to the present invention is ≤ 2.5 mm/a under the corrosion environment conditions of a temperature of 60°C, a CO₂ partial pressure of 1 MPa, and a NaCl concentration of 20 g/L, thus having excellent carbon dioxide corrosion resistance.

### Description of the drawings

FIG. 1 is a photograph of the microstructure of the petroleum casing pipe of Example 1 of the present invention under an optical microscope.
FIG. 2 is a photograph of the microstructure of the petroleum casing pipe of Example 1 of the present invention under a scanning electron microscope.
FIG. 3 is a photograph of the microstructure of the petroleum casing pipe of Comparative Example 1 under a scanning electron microscope.

### Detailed Description

Below, the high-strength petroleum casing pipe resistant to carbon dioxide corrosion and its manufacturing method according to the present invention will be further explained and illustrated in conjunction with specific examples and the drawings of the specification; however, such explanation and illustration shall not unduly limit the technical solution of the present invention.

### Examples 1-18 and Comparative Examples 1-5

The high-strength petroleum casing pipes resistant to carbon dioxide corrosion of Examples 1-18 are all prepared by the following steps:
(1) Smelting: Smelting is performed through primary smelting, secondary refining, and vacuum degassing, with the tapping temperature being 1600-1700°C.
(2) Continuous Casting: Round billets are produced by the continuous casting process. The superheat degree of molten steel is controlled to be ≤ 30°C, and the continuous casting speed is controlled at 2.0 m/min or lower.
(3) Heating and Piercing: The round billets are heated to a soaking temperature of 1200-1250°C in a rotary heating furnace and held for 100-300 minutes, followed by piercing at a temperature of 1150-1250°C.
(4) Rolling: After piercing, continuous rolling is carried out, with the finishing rolling temperature controlled at 900-1000°C.
(5) Sizing: After short-time heating in a heating furnace, sizing is performed, and the sizing temperature is controlled at 850-950°C.
(6) Quenching: Heat to 880-920°C, hold for 30-60 minutes, and then perform water quenching.
(7) Tempering: The tempering temperature is 550-650°C, a holding time is 45-75 minutes, and then air cooling is performed.

It should be noted that the comparative petroleum casing pipes of Comparative Examples 1-5 are prepared with reference to the steps of Examples 1-18, but the chemical element contents and/or process parameters during the manufacturing process of Comparative Examples 1-5 do not meet the design requirements of the present invention.

Table 1 lists the mass percentage ratios of each chemical element in the high-strength petroleum casing pipes resistant to carbon dioxide corrosion of Examples 1-18 and the comparative petroleum casing pipes of Comparative Examples 1-5.

**Table 1. (wt%, with the balance being Fe and other unavoidable impurities except P, S, and N)**

| NO. | C | Si | Mn | P | S | Cr | Mo | Al | V | Ni | Nb | N | Ce | La |
|---|---|---|---|---|---|---|---|---|---|---|---|---|---|---|
| Ex. 1 | 0.15 | 0.25 | 0.5 | 0.008 | 0.002 | 3.0 | 0.5 | 0.03 | 0.15 | 0.5 | - | 0.005 | 0.006 | 0.003 |
| Ex. 2 | 0.10 | 0.15 | 1.5 | 0.005 | 0.004 | 3.0 | 0.6 | 0.04 | 0.13 | 0.4 | - | 0.003 | 0.005 | 0.003 |
| Ex. 3 | 0.20 | 0.3 | 0.4 | 0.007 | 0.002 | 3.2 | 0.1 | 0.1 | 0.15 | 0.4 | - | 0.006 | 0.002 | 0.002 |
| Ex. 4 | 0.16 | 0.6 | 0.2 | 0.007 | 0.003 | 4.0 | 0.4 | 0.06 | 0.15 | 0.5 | - | 0.002 | 0.004 | 0.002 |
| Ex. 5 | 0.14 | 0.8 | 0.1 | 0.010 | 0.003 | 5.0 | 0.2 | 0.05 | 0.19 | 0.4 | - | 0.004 | 0.005 | 0.004 |
| Ex. 6 | 0.17 | 0.4 | 0.6 | 0.011 | 0.002 | 3.5 | 0.3 | 0.01 | 0.16 | 0.1 | - | 0.003 | 0.01 | 0.01 |
| Ex. 7 | 0.18 | 0.1 | 0.8 | 0.009 | 0.002 | 3.3 | 0.7 | 0.02 | 0.12 | 0.3 | - | 0.002 | 0.008 | 0.004 |
| Ex. 8 | 0.12 | 0.25 | 1.2 | 0.008 | 0.004 | 3.1 | 0.6 | 0.01 | 0.1 | 0.5 | - | 0.004 | 0.01 | 0.008 |
| Ex. 9 | 0.11 | 0.75 | 0.4 | 0.006 | 0.004 | 3.1 | 0.4 | 0.05 | 0.17 | 0.4 | - | 0.007 | 0.005 | 0.004 |
| Ex. 10 | 0.14 | 0.3 | 1.0 | 0.010 | 0.001 | 3.3 | 0.5 | 0.03 | 0.1 | 0.3 | - | 0.006 | 0.006 | 0.003 |
| Ex. 11 | 0.16 | 0.1 | 0.3 | 0.005 | 0.002 | 3.4 | 0.5 | 0.1 | 0.2 | 0.4 | 0.01 | 0.003 | 0.003 | 0.002 |
| Ex. 12 | 0.15 | 0.25 | 0.4 | 0.007 | 0.002 | 3.2 | 0.6 | 0.08 | 0.16 | 0.1 | 0.01 | 0.002 | 0.004 | 0.004 |
| Ex. 13 | 0.16 | 0.2 | 1.1 | 0.009 | 0.003 | 3.0 | 0.4 | 0.05 | 0.11 | 1.0 | 0.02 | 0.005 | 0.006 | 0.003 |
| Ex. 14 | 0.15 | 0.2 | 0.9 | 0.008 | 0.003 | 3.2 | 0.4 | 0.03 | 0.12 | 0.3 | 0.02 | 0.004 | 0.002 | 0.002 |
| Ex. 15 | 0.13 | 0.5 | 0.6 | 0.007 | 0.004 | 3.2 | 0.5 | 0.03 | 0.15 | 0.4 | 0.03 | 0.003 | 0.01 | 0.005 |
| Ex. 16 | 0.14 | 0.3 | 1.0 | 0.011 | 0.004 | 3.3 | 0.4 | 0.07 | 0.11 | 0.3 | 0.05 | 0.004 | 0.005 | 0.003 |
| Ex. 17 | 0.15 | 0.3 | 0.4 | 0.010 | 0.004 | 3.0 | 0.3 | 0.02 | 0.15 | 0.7 | 0.10 | 0.005 | 0.009 | 0.005 |
| Ex. 18 | 0.16 | 0.2 | 0.8 | 0.011 | 0.001 | 3.1 | 0.2 | 0.05 | 0.13 | 0.6 | 0.15 | 0.004 | 0.007 | 0.002 |
| Comp. Ex. 1 | *0.35* | 0.25 | 1.1 | 0.012 | 0.002 | 3 | 0.5 | 0.03 | 0.15 | 0.5 | - | 0.005 | 0.006 | 0.003 |
| Comp. Ex. 2 | ***0.35*** | 0.25 | 0.5 | 0.007 | 0.002 | ***1*** | 0.5 | 0.03 | 0.15 | 0.5 | - | 0.003 | 0.006 | 0.003 |
| Comp. Ex. 3 | 0.15 | 0.3 | 0.5 | 0.005 | 0.001 | 3 | - | 0.03 | 0.15 | 0.5 | - | 0.003 | 0.006 | 0.003 |
| Comp. Ex. 4 | 0.15 | 0.2 | 0.3 | 0.006 | 0.004 | 3 | 0.5 | 0.03 | - | 0.5 | 0.01 | 0.002 | - | - |
| Comp. Ex. 5 | 0.15 | 0.25 | 0.5 | 0.007 | 0.003 | 3 | 0.5 | 0.03 | 0.15 | 0.5 | 0.01 | 0.006 | - | - |

Table 2 lists the specific process parameters of the high-strength petroleum casing pipes resistant to carbon dioxide corrosion of Examples 1-18 and the comparative petroleum casing pipes of Comparative Examples 1-5 in the above process steps.

Samples were taken from the high-strength petroleum casing pipes resistant to carbon dioxide corrosion of Examples 1-18 and the comparative pipe materials of Comparative Examples 1-5 respectively. Statistics of large inclusion particles with an average diameter greater than 5 µm and measurement of grain size were performed, and the obtained test results are listed in Table 3. For the statistics of inclusions, with reference to the standard T/CSTM 00346-2021 "Automatic Classification and Statistics of Inclusions in Steel - Scanning Electron Microscope Energy Dispersive Spectrometry Method", the scanning electron microscope energy dispersive spectrometry was used for inclusion analysis to count the size and quantity of inclusions. For the grain size statistics, with reference to the standard GB/T 6394-2017 "Test Methods for Determining Average Grain Size of Metals", the intercept method was adopted for measurement to calculate and determine the grain size grade G.

**Table 3.**

| No. | Percentage by quantity of large inclusions with an average diameter greater than 5µm (%) | Grain size G |
|---|---|---|
| Ex. 1 | 4.86 | 10.5 |
| Ex. 2 | 4.57 | 10.5 |
| Ex. 3 | 3.79 | 11.0 |
| Ex. 4 | 5.10 | 10.0 |
| Ex. 5 | 4.65 | 10.5 |
| Ex. 6 | 5.22 | 10.0 |
| Ex. 7 | 4.49 | 10.5 |
| Ex. 8 | 5.08 | 10.0 |
| Ex. 9 | 4.11 | 11.0 |
| Ex. 10 | 3.65 | 11.0 |
| Ex. 11 | 4.47 | 10.5 |
| Ex. 12 | 5.04 | 10.5 |
| Ex. 13 | 4.55 | 10.5 |
| Ex. 14 | 5.77 | 10.0 |
| Ex. 15 | 3.36 | 11.0 |
| Ex. 16 | 4.92 | 10.5 |
| Ex. 17 | 5.05 | 10.5 |
| Ex. 18 | 4.74 | 10.5 |
| Comp. Ex. 1 | 5.33 | 10.0 |
| Comp. Ex. 2 | 5.14 | 10.5 |
| Comp. Ex. 3 | 5.08 | 10.0 |
| Comp. Ex. 4 | ***16.37*** | ***9.5*** |
| Comp. Ex. 5 | ***15.85*** | ***9.5*** |

As can be seen from Table 3, the grain size of each Example of the present invention is Grade 10 or above, and the percentage by quantity of large inclusions with an average diameter greater than 5 µm in all inclusions is less than 6%. In contrast, the grain size grades of Comparative Examples 4 and 5 are lower than Grade 10, and the proportion of large inclusions is also much higher than that of the Examples of the present invention.

In addition, FIG. 1 shows a microstructural photograph of the petroleum casing pipe of Example 1 of the present invention under an optical microscope. As can be seen from FIG. 1, the metallographic microstructure of Example 1 at room temperature is a tempered sorbite structure. Observation under an optical microscope shows that the microstructures of the petroleum casing pipes of Examples 2-18 are also tempered sorbite.

FIG. 2 shows a microstructural photograph of the petroleum casing pipe of Example 1 of the present invention under a scanning electron microscope. As can be seen from FIG. 2, the microstructure of Example 1 contains a small amount of fine and dispersed carbides. Observation under a scanning electron microscope shows that the microstructures of the petroleum casing pipes of Examples 2-18 also contain a small amount of fine and dispersed carbides.

FIG. 3 shows a microstructural photograph of the petroleum casing pipe of Comparative Example 1 under a scanning electron microscope. As can be seen from FIG. 3, the microstructure of Comparative Example 1 contains a large number of coarse carbides, which are unfavorable to corrosion resistance.

In addition, samples were taken from the high-strength petroleum casing pipes resistant to carbon dioxide corrosion of Examples 1-18 and the comparative pipe materials of Comparative Examples 1-5 respectively for mechanical property tests and corrosion resistance tests, and the test results are listed in Table 4. The relevant test procedures are described as follows:
With reference to the standard GB/T 228.1-2021 "Metallic Materials - Tensile Testing - Part 1: Method of Tensile Testing at Room Temperature", room temperature tensile property tests were conducted to measure the yield strength, tensile strength, and elongation after fracture.

V-notch impact specimens were processed, and with reference to the standard GB/T 229-2020 "Metallic Materials - Charpy Pendulum Impact Test Method", impact property tests at 0°C were performed to determine the impact energy at 0°C.

With reference to the standard JB/T 7901-1999 "Metallic Materials - Laboratory Uniform Corrosion Full Immersion Test Method", samples were taken to process corrosion coupons. Tests were carried out in an autoclave under the following corrosion environment conditions: a temperature of 60°C, a CO₂ partial pressure of 1 MPa, a NaCl concentration of 20 g/L, a rotation speed of 1 m/s, and a test cycle of 168 h. The uniform corrosion rate was calculated. The cross-sections of the corrosion coupons were analyzed by SEM + EDS to determine the Cr content in the corrosion product film.

Table 4 lists the test results of the high-strength petroleum casing pipes resistant to carbon dioxide corrosion of Examples 1-18 and the comparative petroleum casing pipes of Comparative Examples 1-5.

**Table 4.**

| No. | Yield Strength Rp_{0.2} (MPa) | Tensile Strength Rm (MPa) | Elongation after Fracture A (%) | Impact Energy KV8 at 0°C (J) | Uniform Corrosion Rate (mm/a) | Cr Content in Corrosion Product Film (wt%) |
|---|---|---|---|---|---|---|
| Ex. 1 | 1016 | 1176 | 20.5 | 128 | 2.23 | 13.78 |
| Ex. 2 | 990 | 1150 | 19.5 | 124 | 2.15 | 16.47 |
| Ex. 3 | 1128 | 1290 | 20.0 | 85 | 2.49 | 13.33 |
| Ex. 4 | 977 | 1160 | 22.5 | 156 | 1.44 | 17.21 |
| Ex. 5 | 996 | 1181 | 19.5 | 143 | 0.88 | 20.95 |
| Ex. 6 | 988 | 1131 | 22.0 | 146 | 2.28 | 14.43 |
| Ex. 7 | 1030 | 1180 | 20.0 | 119 | 2.18 | 15.35 |
| Ex. 8 | 970 | 1128 | 19.5 | 142 | 2.25 | 13.84 |
| Ex. 9 | 1165 | 1287 | 20.0 | 86 | 2.19 | 14.37 |
| Ex. 10 | 1006 | 1183 | 21.5 | 131 | 2.24 | 15.74 |
| Ex. 11 | 1084 | 1247 | 21.0 | 92 | 2.22 | 13.28 |
| Ex. 12 | 1109 | 1254 | 19.5 | 87 | 2.45 | 15.73 |
| Ex. 13 | 985 | 1135 | 22.0 | 142 | 2.03 | 14.90 |
| Ex. 14 | 1029 | 1181 | 19.0 | 111 | 2.27 | 15.08 |
| Ex. 15 | 972 | 1135 | 22.5 | 178 | 2.20 | 13.61 |
| Ex. 16 | 1023 | 1183 | 23.5 | 134 | 2.23 | 15.73 |
| Ex. 17 | 1113 | 1291 | 22.0 | 129 | 2.25 | 13.05 |
| Ex. 18 | 975 | 1138 | 21.5 | 188 | 2.16 | 14.22 |
| Comp. Ex. 1 | 1127 | 1287 | 19.0 | 63 | **3.27** | **2.05** |
| Comp. Ex. 2 | 998 | 1040 | 23.5 | 97 | ***6.09*** | ***0.79*** |
| Comp. Ex. 3 | ***951*** | 1095 | 22.5 | 124 | ***2.84*** | ***11.57*** |
| Comp. Ex. 4 | ***884*** | 1035 | 23.0 | 89 | ***2.95*** | ***9.58*** |
| Comp. Ex. 5 | 962 | 1213 | 21.5 | 81 | ***2.91*** | ***10.24*** |

As can be seen from Table 4, the yield strength of the high-strength petroleum casing pipes resistant to carbon dioxide corrosion according to Examples 1-18 of the present invention is all higher than 965 MPa, the tensile strength is all higher than 1034 MPa, and the transverse Charpy impact energy at 0°C is all greater than 80 J. Meanwhile, under the test corrosion environment, the Cr content in the corrosion product film of each Example of the present invention is higher than 13 wt%, and the uniform corrosion rate is all lower than 2.5 mm/a.

However, because the chemical element contents of Comparative Examples 1-5 do not meet the design requirements of the present invention, their corrosion resistance is inferior to that of the present invention, and their mechanical properties are also poor.

It can thus be seen that by adopting the technical scheme described in the present invention, a petroleum casing pipe with both ultra-high strength and carbon dioxide corrosion resistance can be obtained.

It should be noted that the combination modes of various technical features in the present invention are not limited to the combination modes recorded in the claims of the present invention or the combination modes recorded in the specific embodiments. All technical features recorded in the present invention may be freely combined or integrated in any manner unless they contradict each other.

It should also be noted that the Examples listed above are only specific embodiments of the present disclosure. Obviously, the present disclosure is not limited to the above Examples, and changes or modifications made thereto can be directly derived from the present disclosure or easily conceived of by those skilled in the art, all of which fall within the protection scope of the present disclosure.

## Claims

1. A high-strength petroleum casing pipe resistant to carbon dioxide corrosion, comprising Fe and unavoidable impurities, wherein the petroleum casing pipe further comprises the following chemical elements in mass percentage: C: 0.10~0.20%, Si: 0.10~0.80%, Mn: 0.10~1.50%, Cr: 3~5%, Mo: 0.10~0.70%, Al: 0.01~0.10%, V: 0.10~0.20%, Ni: 0.1~1.0%, Ce: 0.002~0.01%, and La: 0.002~0.01 %.

2. The high-strength petroleum casing pipe resistant to carbon dioxide corrosion according to claim 1, wherein the petroleum casing pipe comprises the following chemical elements in mass percentage: C: 0.10~0.20%, Si: 0.10~0.80%, Mn: 0.10~1.50%, Cr: 3~5%, Mo: 0.10~0.70%, Al: 0.01~0.10%, V: 0.10~0.20%, Ni: 0.1~1.0%, Ce: 0.002~0.01%, La: 0.002~0.01%, and a balance of Fe and other unavoidable impurities.

3. The high-strength petroleum casing pipe resistant to carbon dioxide corrosion according to claim 1 or 2, wherein the mass percentages of the chemical elements in the petroleum casing pipe further satisfy at least one of the following:
Si: 0.1~0.4%;
Mn: 0.2~1.0%;
Mo: 0.4~0.6%;
Al: 0.01~0.04%;
Ni: 0.1~0.5%;
Ce: 0.002~0.008%; and
La: 0.002~0.005%.

4. The high-strength petroleum casing pipe resistant to carbon dioxide corrosion according to claim 1 or 2, wherein the petroleum casing pipe further comprises 0 < Nb ≤ 0.15wt%.

5. The high-strength petroleum casing pipe resistant to carbon dioxide corrosion according to claim 1 or 2, wherein among the unavoidable impurities: P ≤ 0.015%, S ≤ 0.008%, and N ≤ 0.008%.

6. The high-strength petroleum casing pipe resistant to carbon dioxide corrosion according to claim 1 or 2, wherein a matrix microstructure of the petroleum casing pipe is tempered sorbite.

7. The high-strength petroleum casing pipe resistant to carbon dioxide corrosion according to claim 1 or 2, wherein a grain size of the petroleum casing pipe is Grade 10 or above.

8. The high-strength petroleum casing pipe resistant to carbon dioxide corrosion according to claim 1 or 2, wherein a percentage by quantity of large inclusions with an average diameter greater than 5µm in all inclusions is < 6%.

9. The high-strength petroleum casing pipe resistant to carbon dioxide corrosion according to claim 1 or 2, wherein a Cr content in a corrosion product film of the petroleum casing pipe is higher than 13wt%.

10. The high-strength petroleum casing pipe resistant to carbon dioxide corrosion according to claim 1 or 2, wherein the properties of the petroleum casing pipe satisfy: a yield strength of 965~1173MPa, a tensile strength ≥ 1034MPa, and a transverse Charpy impact energy at 0°C ≥ 80J.

11. The high-strength petroleum casing pipe resistant to carbon dioxide corrosion according to claim 1 or 2, wherein a uniform corrosion rate of the petroleum casing pipe is ≤ 2.5mm/a under corrosion environment conditions of a temperature of 60°C, a CO₂ partial pressure of 1MPa, and a NaCl concentration of 20g/L.

12. A method for manufacturing the high-strength petroleum casing pipe resistant to carbon dioxide corrosion according to any one of claims 1-11, wherein the method comprises the following steps:
(1) smelting and continuous casting to obtain a pipe billet;
(2) heating, piercing, rolling, and sizing;
(3) quenching: heating to a quenching temperature of 880~920°C, holding for 30-60 minutes, followed by water quenching;
(4) tempering: heating to a tempering temperature of 550~650°C, with a holding time of 45~75 minutes.

13. The manufacturing method according to claim 12, wherein in step (1), during the casting process, a superheat degree of molten steel is controlled to be ≤ 30°C, and a continuous casting speed is controlled at 2.0m/min or lower.

14. The manufacturing method according to claim 12, wherein in step (2), the pipe billet is heated to a soaking temperature of 1200~1250°C and held for 100~300 minutes.

15. The manufacturing method according to claim 12, wherein the manufacturing method has one or more of the following characteristics:
in step (2), a piercing temperature is controlled at 1150~1250°C;
in step (2), a finishing rolling temperature is controlled at 900~1000°C;
in step (2), a sizing temperature is controlled at 850-950°C.
